

# UNITED STATES PATENT OFFICE.

ROBERT MCKNIGHT, OF PITTSBURGH, PENNSYLVANIA.

## PROCESS OF MAKING COMPOUNDS OF RARE METALS.

1,308,911.

Specification of Letters Patent.

Patented July 8, 1919.

No Drawing. Application filed October 4, 1912, Serial No. 723,992. Renewed November 7, 1918. Serial No. 261,551.

To all whom it may concern:

Be it known that I, ROBERT MCKNIGHT, a citizen of the United States, residing at Pittsburgh, in the county of Allegheny and State of Pennsylvania, have invented a certain new and useful Process of Making Compounds of Rare Metals, of which the following is a specification.

The invention relates to the process of making compounds including the rare metals such as tungsten, uranium, vanadium, molybdenum, and tellurium. It is well known that the addition of various amounts of the rare metals improve iron, steel, and other of the more common metals when added in the proper proportions, but these rare metals are now commonly produced in a metallic condition and require very high melting points before the desired combination can be accomplished. It is the primary objects of the present invention to provide a process whereby the incorporation of the rare metals with the other more common metals is accomplished at a much lower temperature than has heretofore been possible; the provision of a process in which the desired combination between the rare metal and the common metal occurs at the ordinary melting point of the common metal; and the provision of a process wherein the melting point of the compound to which the rare metal has been added is reduced below that of the common metal prior to the addition of the rare metal, such as is not the case with the ordinary metallic compounds of the rare and common metals as now produced.

In carrying out the process I employ the acid or alkaline salts of the rare metals, which salts may be obtained in any manner known in the art, a desirable method being set forth in my Patent Number 862,987 of August 13, 1907. A specific instance of one manner of practising my invention is as follows: Taking a salt containing tungstic acid ( $WO_3$ ) as the rare metal salt, I mix such salt with one of the haloid salts, such as sodium chlorid, and feed the mixture into a furnace of any desired type, it being understood however, that if desired, the two compounds may be fed into the furnace separately and there mixed. The amount or proportion of sodium chlorid may be varied, the desired result being more quickly obtained with the larger portion of the sodium chlorid. I find in practice however, that

the advantage derived from a large excess of sodium chlorid, such as would be expected from the law of mass action, is after a certain point counterbalanced by the disadvantage of having to handle too large a bulk of material, and therefore the amount of sodium chlorid to be used is best determined by the amount of rare metal in the rare metal salt. I find that with a salt containing 90% of tungstic oxid, 20% of sodium chlorid gives excellent results. The temperature applied need not exceed 800° C. which can be secured through any available fuel. Where electricity is available a good furnace in which to carry out the process is set forth in my Patent Number 900,192 of October 6, 1908. As a result of this treatment the tungstic acid combines with the sodium chlorid and forms when cooled a hard semimetallic cake or ingot.

The compound as just described is supplied with the common metal to be modified in quantities sufficient to give the quality desired for any specific purpose such as for instance the making of high speed tools where the common metal is steel, the combination with the steel occurring at a temperature approximately the melting point of the steel, and the heat for melting the steel being supplied in any of the known ways.

It will be understood that the invention is not limited to the specific application of the method as heretofore explained for the purpose of illustration. The other haloid salts might be employed, although not so desirable, and more expensive than sodium chlorid. Similarly the invention is applicable to use with other of the common metals than iron or steel, and the proportions of the materials employed might be varied within considerable limits. The resultant compound of the rare metal salt and the haloid salt is, as a matter of convenience, preferably allowed to cool and harden after uniting, but if desired, it may be used as a liquid, the result when the compound is used as a liquid being the same as when used as a solid. I believe the composition, whether in solid or liquid form, to be a true chemical compound, rather than a mechanical mixture, but as yet I have been unable to determine the exact character of the reactions involved. The composition as a solid is dark, very dense, has a decided me-

tallic appearance, and discloses no free sodium chlorid.

In the application of the process to the modification of steel by the rare metal the primary advantages of my method over the methods now in use may be summed up as follows. First, the time required to secure the incorporation of the rare metal into the steel is reduced by reason of the fact that 10 the steel need not be heated within many hundred degrees of the temperature required under the present practice, the union of the rare metal occurring at the melting temperature of the steel and within a few 15 minutes, thus involving a great saving in time; second, the cost of fuel is correspondingly reduced, and third, the loss of steel due to burning is entirely eliminated.

Having thus described my invention, 20 what I claim as new and desire to secure by Letters Patent, is the following:

1. The process of making compounds of the rare metals, such as tungsten, vanadium, uranium, molybdenum and tellurium, which

consists in melting together a salt of the 25 rare metal and a chlorid of one of the alkali metals without any substantial volatilization of the rare metal.

2. The process of making compounds of the rare metals, such as tungsten, vanadium, 30 uranium, molybdenum and tellurium, which consists in melting together a salt of the rare metal and a chlorid of one of the alkali metals, after which the mixture is allowed to cool and harden into a solid body. 35

3. A compound formed by melting together a salt of the rare metals, such as tungsten, vanadium, uranium, molybdenum and tellurium, and a chlorid of one of the alkali metals at a temperature approxi- 40 mately 800 degrees C.

In testimony whereof I have hereunto signed my name in the presence of the two subscribed witnesses.

ROBERT McKNIGHT.

Witnesses:

LETITIA A. MYERS,  
ARCHWORTH MARTIN.